# EUROPEAN PATENT SPECIFICATION

(11) **EP 3 932 580 B1**
(45) Date of publication and mention of the grant of the patent: **06.03.2024**
(21) Application number: 21181766.3
(22) Date of filing: 25.06.2021
(51) Int. Cl.: B21D 22/16, B21D 53/30, B22D 21/00, B23P 15/00

(54) **METHOD OF PRODUCING A WHEEL FOR STRADDLED VEHICLES**
VERFAHREN ZUR HERSTELLUNG EINES RADS FÜR GRÄTSCHSITZFAHRZEUGE
PROCÉDÉ DE PRODUCTION D'UNE ROUE POUR VÉHICULES À CALIFOURCHON

(30) Priority: 29.06.2020 JP 2020112092; 31.08.2020 JP 2020145282
(43) Date of publication of application: 05.01.2022
(73) Proprietor: Yamaha Hatsudoki Kabushiki Kaisha, Iwata-shi, Shizuoka 438-8501 (JP)
(72) Inventor: SUENAGA, Kentaro, Shizuoka, 438-8501 (JP); KURIMOTO, Yukihiro, Shizuoka, 438-8501 (JP); SUZUKI, Yasunobu, Shizuoka, 438-8501 (JP); MATSUBARA, Keisuke, Shizuoka, 438-8501 (JP); KASHIMA, Hitoshi, Shizuoka, 438-8501 (JP); FUKUJI, Hidehiro, Shizuoka, 438-8501 (JP); NAGAYAMA, Jun, Shizuoka, 438-8501 (JP); OSHIMA, Kahori, Shizuoka, 438-8501 (JP)
(74) Representative: Grünecker Patent- und Rechtsanwälte PartG mbB

(56) References cited:
- EP-A1- 0 765 700
- CN-U- 209 439 701
- JP-A- 2002 254 133
- US-A- 4 624 038
- Flowform Wheels: "FlowForm Wheels | A Look Inside The Factory", , 7 May 2020 (2020-05-07), XP055859085, Retrieved from the Internet: URL:https://www.youtube.com/watch?v=C6nMHW sWPMg [retrieved on 2021-11-09]

## Description

The present invention relates to a method of producing a wheel for straddled vehicles.

In recent years, along with steels, aluminum alloys are widely used as the material of wheels for automotive vehicles.

Prior art document US 4,624,038 discloses a method of producing a wheel from aluminum alloy. The wheel includes a hub having an aperture into which a wheel shaft is to be inserted, an annular rim, and a plurality of spokes connecting the hub and the rim. The method comprising:
step A of forming an intermediate product from an aluminum alloy by using a casting technique, the intermediate product including a precursory hub, an annular precursory rim, and a plurality of precursory spokes connecting the precursory hub (110') and the precursory rim;
step B of performing a shear-forming operation as a flow forming process for the precursory rim of the intermediate product by using a flow forming apparatus, wherein, while the intermediate product is rotated, at least a portion of the precursory rim is drawn in a first direction and a second direction, the first direction being one direction that extends from a center of the intermediate product on an axial direction of the intermediate product, and the second direction being an opposite direction that extends from the center of the intermediate product on the axial direction of the intermediate product; and the precursory rim comprises annular wing portions which project in opposite axial directions from a disc portion. With said shear-forming operation, the wing portions are reduced in thickness by about 25% to 50% to form a thinner and wider rim portion.

JP 5205655 B2 discloses a method of producing a wheel made of an aluminum alloy, where a tilting gravity casting apparatus is used. Employing a gravity casting technique for producing a wheel is advantageous in terms of reducing the weight of relatively large wheels because it is easy to form a hollow structure by utilizing a core.

However, when producing a wheel made of an aluminum alloy by using a gravity casting technique, some improvement could still be made in the material strength (mechanical properties) of the rim, in which solidification tends to be slow and defects are likely to remain.

The present invention has been made in view of the above problem, and an objective thereof is to provide a method of producing a wheel for straddled vehicles that is able to adequately improve the mechanical properties of a rim. According to the present invention said object is solved by a method of producing a wheel for straddled vehicles having the features of independent claim 1. Preferred embodiments are laid down in the dependent claims.

### BRIEF DESCRIPTION OF THE DRAWINGS

FIG. 1 is a left side view schematically showing a wheel 100 for straddled vehicles.
FIG. 2 is a right side view schematically showing the wheel 100.
FIG. 3 is a plan view showing the wheel 100 as viewed from a radial direction.
FIG. 4 is a flowchart showing an example of a method of producing the wheel 100.
FIG. 5 is a left side view schematically showing an intermediate product (workpiece) 100'.
FIG. 6 is a right side view schematically showing the workpiece 100'.
FIG. 7 is a plan view showing the workpiece 100' as viewed from a radial direction.
FIG. 8 is a cross-sectional view taken along line 8A-8A' in FIG. 5.
FIG. 9 is a diagram schematically showing a flow forming apparatus 10.
FIG. 10A is a left side view schematically showing the workpiece 100' after a flow forming process.
FIG. 10B is a right side view schematically showing the workpiece 100' after a flow forming process.
FIG. 10C is a plan view showing the workpiece 100' after a flow forming process as viewed from a radial direction.
FIG. 10D is a cross-sectional view taken along line 10D-10D' in FIG. 10A.
FIG. 11 is a cross-sectional view taken along line 11A-11A' in FIG. 1.
FIG. 12A is a diagram showing an example positioning of a knockout ring 24.
FIG. 12B is a diagram showing another example positioning of the knockout ring 24.
FIG. 13 is a left side view schematically showing the workpiece 100'.
FIG. 14 is a right side view schematically showing the workpiece 100'.
FIG. 15 is a cross-sectional view taken along line 15A-15A' in FIG. 13.
FIG. 16 is a cross-sectional view taken along line 16A-16A' in FIG. 13.
FIG. 17 is a side view schematically showing a lower mandrel 21 and an upper mandrel 22.
FIG. 18 is a cross-sectional view schematically showing a state where the workpiece 100' is clamped by the lower mandrel 21 and the upper mandrel 22.
FIG. 19 is a left side view schematically showing the workpiece 100' after a flow forming process.
FIG. 20 is a right side view schematically showing the workpiece 100' after a flow forming process.
FIG. 21 is a left side view schematically showing the workpiece 100'.
FIG. 22 is a right side view schematically showing the workpiece 100'.
FIG. 23 is a left side view schematically showing the workpiece 100'.
FIG. 24 is a right side view schematically showing the workpiece 100'.
FIG. 25 is a cross-sectional view taken along line 25A-25A' in FIG. 23.
FIG. 26 is a cross-sectional view taken along line 26A-26A' in FIG. 23.
FIG. 27 is a graph showing a relationship between the percentage content of Si and tensile strength and proof stress for Examples 1 to 3 and Reference Example 3.
FIG. 28 is a graph showing a relationship between the percentage content of Si and elongation for Examples 1 to 3 and Reference Example 3.
FIG. 29 is a graph showing a relationship between the percentage content of Mg and tensile strength and proof stress for Examples 3 to 7 and Reference Examples 4 and 5.
FIG. 30 is a graph showing a relationship between the percentage content of Mg and elongation for Examples 3 to 7 and Reference Examples 4 and 5.
FIG. 31 is a graph showing a relationship between the percentage content of Cu and tensile strength and proof stress for Examples 3, 8 and 9.
FIG. 32 is a graph showing a relationship between the percentage content of Cu and elongation for Examples 3, 8 and 9.
FIG. 33 is a graph showing a relationship between the percentage content of Fe and tensile strength and proof stress for Examples 3, 10 and 11.
FIG. 34 is a graph showing a relationship between the percentage content of Fe and elongation for Examples 3, 10 and 11.
FIG. 35 is a graph showing a relationship between the percentage content of Ti and tensile strength and proof stress for Examples 3, 12 and 13.
FIG. 36 is a graph showing a relationship between the percentage content of Ti and elongation for Examples 3, 12 and 13.
FIG. 37 is a graph showing a relationship between the percentage content of Na and tensile strength and proof stress for Examples 14 to 17.
FIG. 38 is a graph showing a relationship between the percentage content of Na and elongation for Examples 14 to 17.
FIG. 39 is a graph showing a relationship between the percentage content of Sr and tensile strength and proof stress for Examples 3, 14, and 18 to 20.
FIG. 40 is a graph showing a relationship between the percentage content of Sr and elongation for Examples 3, 14, and 18 to 20.

### DETAILED DESCRIPTION

Hereinafter, embodiments of the present teaching will be described with reference to the drawings.

### [vehicle wheel]

With reference to FIGS. 1 to 3, an example of a wheel for straddled vehicles (hereinafter simply referred to as a "wheel") that is produced by a production method according to an embodiment of the present teaching will be described. FIGS. 1 and 2 are a left side view and a right side view, respectively, schematically showing the wheel 100. FIG. 3 is a plan view showing the wheel 100 from a radial direction.

As shown in FIGS. 1, 2 and 3, the wheel 100 includes a hub 110, a rim 120, and a plurality of spokes 130. The wheel 100 is made of a metal material. The hub 110, the rim 120, and the plurality of spokes 130 are monolithically formed.

The hub 110 is located in the center of the wheel 100, and has an aperture (wheel-shaft insertion hole) 111, into which a wheel shaft is to be inserted. A direction that is parallel to a center axis of the wheel-shaft insertion hole 111 may be referred to as the "axial direction" hereinbelow. Note that the specific shape of the hub 110 is not limited to what is illustrated in FIG. 1, etc.

The rim 120 has an annular shape, and extends along the circumferential direction of the wheel 100. The rim 120 has an inner peripheral surface 120a and an outer peripheral surface 120b. A tire is to be mounted on the outer peripheral surface 120b of the rim 120.

The plurality of spokes 130 connect the hub 110 and the rim 120. More specifically, the plurality of spokes 130 connect an outer periphery of the hub 110 and the inner peripheral surface 120a of the rim 120. Although the example shown illustrates the wheel 100 as having ten spokes 130, the number of spokes 130 is not limited to ten. Although the example shown illustrates that two adjacent spokes 130 are united at the hub 110 side, the configuration of the spokes 130 is not limited thereto.

### [Method of producing a wheel for straddled vehicles]

With reference to FIG. 4, a method of producing the wheel 100 will be described. FIG. 4 is a flowchart showing an example of a method of producing the wheel 100.

First, by using a gravity casting technique, an intermediate product (hereinafter referred to as a "workpiece") 100' is formed from an aluminum alloy (Step s1). Specific shapes for the workpiece 100' are shown in FIG. 5 to FIG. 8. FIG. 5 and FIG. 6 are a left side view and a right side view, respectively, schematically showing the workpiece 100'. FIG. 7 is a plan view showing the workpiece 100' as viewed from a radial direction. FIG. 8 is a cross-sectional view taken along line 8A-8A' in FIG. 5.

As shown in FIG. 5 to FIG. 7, the workpiece 100' includes a precursory hub 110', a precursory rim 120', and a plurality of precursory spokes 130' connecting the precursory hub 110' and the precursory rim 120'. The precursory hub 110' is a portion to become the hub 110 of the wheel 100. Similarly, the precursory rim 120' is a portion to become the rim 120, and the precursory spokes 130' are portions to become the spokes 130.

The precursory hub 110' is located at the center of the workpiece 100'. In the example shown, the wheel-shaft insertion hole 111 is not formed in the precursory hub 110' yet. The precursory rim 120' has an annular shape, and extends along the circumferential direction of the workpiece 100'. The precursory rim 120' has an inner peripheral surface 120a' and an outer peripheral surface 120b'. The plurality of precursory spokes 130' connect the precursory hub 110' and the precursory rim 120'. More specifically, the plurality of precursory spokes 130' connect an outer periphery of the precursory hub 110' and the inner peripheral surface 120a' of the precursory rim 120'.

Then, a flow forming process is performed for the precursory rim 120' of the workpiece 100' by using a flow forming apparatus (Step s2). In this Step s2, while the workpiece 100' is rotated, at least a portion of the precursory rim 120' is drawn in a first direction D1, which is one direction that extends from the center of the workpiece 100' on its axial direction (see FIG. 8) and in a second direction D2, which is an opposite direction that extends from the center of the workpiece 100' on its axial direction (see FIG. 8).

An example of a flow forming apparatus to be used at Step s2 is shown in FIG. 9. The flow forming apparatus 10 shown in FIG. 9 includes: a first mandrel 21 and a second mandrel 22; a rotating mechanism 31 to rotate the first mandrel 21 and the second mandrel 22; and a roller 41 to be pressed against the outer peripheral surface 120b' of the precursory rim 120' of the workpiece 100'.

Hereinafter, between the first mandrel 21 and the second mandrel 22, the first mandrel 21 being located relatively low will be referred to as the "lower mandrel", whereas the second mandrel 22 being located relatively high will be referred to as the "upper mandrel".

The rotating mechanism 31, which includes a motor, is placed on a pedestal 11. The lower mandrel 21 is attached to a leading end of the rotating mechanism 31. On a roof 12, a mandrel moving mechanism 32 to move the upper mandrel 22 up or down is placed. The upper mandrel 22 is attached to a leading end of the mandrel moving mechanism 32. On a wall 13, a roller moving mechanism 33 to move the roller 41 in the up-down direction, the right-left direction, or the front-rear direction is placed. The roller 41 is supported, in a rotatable manner, by an arm 42 that is attached to a leading end of the roller moving mechanism 33.

With the workpiece 100' being externally fitted on the lower mandrel 21 and the upper mandrel 22, a flow forming process is performed. At this time, the lower mandrel 21 and the upper mandrel 22 are coupled in such a manner that the upper mandrel 22 will rotate as the lower mandrel 21 rotates. For example, the flow forming process may be performed in a state where a portion the lower mandrel 21 is fitted in a portion of the upper mandrel 22.

The lower mandrel 21 has a surface (hereinafter referred to as the "first abutting surface") 21a that abuts with the inner peripheral surface 120a' of the precursory rim 120' of the workpiece 100' from one direction (e.g., from below herein) along the axial direction of the workpiece 100'.

The upper mandrel 22 has a surface (hereinafter referred to as the "second abutting surface") 22a that abuts with the inner peripheral surface 120a' of the precursory rim 120' of the workpiece 100' from the opposite direction (e.g., from above herein) along the axial direction of the workpiece 100'.

When the lower mandrel 21 and the upper mandrel 22 are rotated by the rotating mechanism 31, the workpiece 100' rotates accordingly. As the roller 41 is pressed against the outer peripheral surface 120b' of the precursory rim 120' of the workpiece 100' in this state, the flow forming process is accomplished.

The workpiece 100' after the flow forming process is shown in FIGS. 10A, 10B, 10C, and 10D. FIG. 10A and FIG. 10B are a left side view and a right side view, respectively, schematically showing the workpiece 100' after the flow forming process. FIG. 10C is a plan view showing the workpiece 100' after the flow forming process as viewed from a radial direction. FIG. 10D is a cross-sectional view taken along line 10D-10D' in FIG. 10A. As shown in FIGS. 10A, 10B, 10C, and 10D, the flow forming process has caused plastic deformation of the precursory rim 120'; more specifically, the precursory rim 120' has been stretched along the axial direction while being also thinned.

Next, a heat treatment is performed. More specifically, a solution treatment (Step s3), a quenching process (Step s4), and an artificial aging process (Step s5) are performed in this order. This series of processes may sometimes be called a T6 heat treatment. The solution treatment may be performed at 530°C for 4.5 hours, for example. The quenching process may be performed through water-cooling at 60°C, for example. The artificial aging process may be performed at 170°C for 3.2 hours, for example.

Thereafter, a cutting process is performed for the workpiece 100', thereby at least completing the rim 120 (Step s6). Through the cutting process, the wheel-shaft insertion hole 111 and the like are formed, and also their dimensions are adjusted. In this manner, the wheel 100 is obtained. FIG. 11 shows a cross section taken along line 11A-11A' in FIG. 1. In the present embodiment, a ratio of the wall thickness t1 (see FIG. 10D) of the precursory rim 120' after Step s2 and before Step s6 to the wall thickness t2 (see FIG. 11) of the rim 120 after Step s6 (hereinafter denoted as the "wall thickness ratio t1/t2") is set within a predetermined range. Note that the "wall thickness ratio" refers to the ratio of wall thicknesses taken at the same place (or site). Note that the wheel-shaft insertion hole 111 does not need to be formed via a cutting process. For example, at step S1, a workpiece 100' that already has a wheel-shaft insertion hole 111 may be provided.

As described above, in the method of producing the wheel 100 according to an embodiment of the present teaching, after Step s1 of forming an intermediate product from an aluminum alloy by a gravity casting technique, Step s2 of performing a flow forming process for a precursory rim of the intermediate product is performed. As a result of this, mechanical properties of the rim 120 can be adequately improved.

Moreover, in the method of producing the wheel 100 according to an embodiment of the present teaching, the wall thickness ratio t1/t2 is set within a predetermined range. Specifically, the percentage wall thickness ratio t1/t2 is not less than 132% and not more than 433%. As a result, while suitably realizing a desired product shape, the efficiency of material use can be enhanced. Hereinafter, this point will be described in detail.

Assuming a cut margin a [mm] in Step s6 (cutting process), the wall thickness t1 is expressed as t1=t2+a, and therefore the wall thickness ratio t1/t2 is expressed as t1/t2=1+a/t2. If the cut margin a is less than 3.0 mm, it may be difficult to realize a desired product shape. On the other hand, if the cut margin exceeds 5.0 mm, the efficiency of use of the material (which herein is an aluminum alloy) is somewhat decreased. Therefore, when one assumes a minimum product wall thickness t2min [mm] and a maximum product wall thickness t2max [mm], it may be said that the wall thickness ratio t1/t2 preferably satisfies the relationship 1+3/t2max ≤ t1/t2 ≤ 1+5/t2min. Herein, given that the minimum product wall thickness t2min is 1.5 mm and that the maximum product wall thickness t2max is 9.5 mm, the wall thickness ratio t1/t2 is preferably not less than 132% and not more than 433%, as is calculated from the above equation.

Thus, because of the wall thickness ratio t1/t2 being not less than 132% and not more than 433%, while suitably realizing a desired product shape, the efficiency of material use can be enhanced.

From the standpoint of adequately improving the mechanical properties of the rim 120 through the flow forming process, Step s2 is preferably performed in such a manner that, in at least a portion of the precursory rim 120', a ratio of the wall thickness t1 of the precursory rim 120' after Step s2 and before Step s6 to the wall thickness t0 of the precursory rim before Step s2 (see FIG. 8) is 50% or less.

Moreover, as in the above-described production method, Step s3 of performing a solution treatment after the flow forming process of Step s2, Step s4 of performing a quenching process after Step s3, and Step s5 of performing an artificial aging process after Step s4 may further be included. This series of heat treatment processes allows the mechanical properties of the wheel 100 made of an aluminum alloy to be adjusted (e.g., so that it increases in tensile strength, proof stress, and hardness).

As shown in FIG. 12A, the flow forming apparatus 10 may further include a knockout ring 24 located at an outer periphery of the first mandrel 21. The knockout ring 24 is able to move up and down. The knockout ring 24 allows the workpiece 100' after the flow forming process to be released from the first mandrel 21.

Given a reference plane p, which is an imaginary plane that is defined by one end face of the workpiece 100' after the flow forming process along the axial direction, an end face (upper surface) of the knockout ring 24 is essentially flush with this reference plane p in the example shown in FIG. 12A; however, the position of the end face of the knockout ring 24 is not limited thereto. As shown in FIG. 12B, the end face of the knockout ring 24 may be offset from the reference plane p along the first direction D1. This will restrain the precursory rim 120' from abutting with the end face of the knockout ring 24 during the flow forming process, thus making it easier for the precursory rim 120' to undergo sufficient plastic deformation. Herein, an amount of offset a of the knockout ring 24 from the reference plane p is preferably set in accordance with a ratio L1/L2 of a length L1 of the precursory rim 120' after Step s2 and before Step s6 as taken along the axial direction (see FIG. 10D) to a length L2 of the rim 120 after Step s6 as taken along the axial direction (see FIG. 11). Specifically, it is preferable that the amount of offset a increases as the ratio L1/L2 increases. Preferably, the ratio L1/L2 is set to not less than 101% and not more than 113%.

### [Another example method of producing a wheel for straddled vehicles]

Another example method of producing the wheel 100 will be described.

First, an intermediate product (workpiece) made of an aluminum alloy is provided. The workpiece may suitably be formed by a gravity casting technique, for example. Specific shapes for the workpiece are shown in FIG. 13 to FIG. 16. FIG. 13 and FIG. 14 are a left side view and a right side view, respectively, schematically showing the workpiece 100'. FIG. 15 and FIG. 16 are cross-sectional views taken along line 15A-15A' and line 16A-16A', respectively, in FIG. 13.

As shown in FIG. 13 to FIG. 16, the workpiece 100' includes a precursory hub 110', a precursory rim 120', and a plurality of precursory spokes 130' connecting the precursory hub 110' and the precursory rim 120'. The precursory hub 110' is a portion to become the hub 110 of the wheel 100. Similarly, the precursory rim 120' is a portion to become the rim 120, and the precursory spokes 130' are portions to become the spokes 130.

The precursory hub 110' is located at the center of the workpiece 100'. In the example shown, the wheel-shaft insertion hole 111 is not formed in the precursory hub 110' yet. The precursory rim 120' has an annular shape, and extends along the circumferential direction of the workpiece 100'. The precursory rim 120' has an inner peripheral surface 120a' and an outer peripheral surface 120b'. The plurality of precursory spokes 130' connect the precursory hub 110' and the precursory rim 120'. More specifically, the plurality of precursory spokes 130' connect an outer periphery of the precursory hub 110' and the inner peripheral surface 120a' of the precursory rim 120'.

Then, a flow forming process is performed for the precursory rim 120' of the workpiece 100' by using a flow forming apparatus. At this step, the flow forming apparatus illustrated in FIG. 9 can be used.

As shown in FIG. 15 and FIG. 16, the inner peripheral surface 120a' of the precursory rim 120' of the workpiece 100' includes: a first region R1 to abut with a first abutting surface 21a of the lower mandrel 21; and a second region R2 to abut with a second abutting surface 22a of the upper mandrel 22. As shown in FIG. 13, FIG. 14 and FIG. 16, each of the first region R1 and the second region R2 includes at least one stepped portion (protrusion) 121 protruding inwardly along the radial direction of the workpiece 100'. In the example shown, each of the first region R1 and the second region R2 includes a plurality of (i.e., two or more) stepped portions 121 that are formed discretely along the circumferential direction of the workpiece 100'.

In the configuration illustrated herein, the stepped portions 121 in the first region R1 and the stepped portions 121 in the second region R2 overlap one another when viewed along the axial direction; however, the positioning of the stepped portions 121 is not limited thereto. Alternatively, the stepped portions 121 in the first region R1 and the stepped portions 121 in the second region R2 may be shifted from one another when viewed along the axial direction (i.e., so that the stepped portions 121 in the first region R1 and the stepped portions 121 in the second region R2 are staggered along the circumferential direction). Although an example has been illustrated where essentially the entire inner peripheral surface 120a' of the precursory rim 120' consists of the first region R1 and the second region R2, the positioning of the first region R1 and the second region R2 is not limited thereto. Alternatively, only a portion of a half of the inner peripheral surface 120a' along the axial direction (i.e., a lower half in FIG. 15 and FIG. 16) may be the first region R1, while only a portion of another half of the inner peripheral surface 120a' along the axial direction (i.e., an upper half in FIG. 15 and FIG. 16) may be the second region R2.

FIG. 17 and FIG. 18 show specific examples of the lower mandrel 21 and the upper mandrel 22. FIG. 17 is a side view schematically showing the lower mandrel 21 and the upper mandrel 22, illustrating a state where the lower mandrel 21 and the upper mandrel 22 are coupled (more specifically, a guide pin 25 of the lower mandrel 21 is inserted in an aperture of the upper mandrel 22). FIG. 18 is a cross-sectional view schematically showing a state where the workpiece 100' is clamped by the lower mandrel 21 and the upper mandrel 22.

As has already been described, the lower mandrel 21 has the first abutting surface 21a, which abuts with the inner peripheral surface 120a' of the precursory rim 120' from below; and the upper mandrel 22 has the second abutting surface 22a, which abuts with the inner peripheral surface 120a' of the precursory rim 120' from above. Each of the first abutting surface 21a of the lower mandrel 21 and the second abutting surface 22a of the upper mandrel 22 is shaped so as to correspond to the plurality of stepped portions 121 of the workpiece 100'. Specifically, each of the first abutting surface 21a of the lower mandrel 21 and the second abutting surface 22a of the upper mandrel 22 includes a plurality of engaging portions (recesses) 23 to engage with the plurality of stepped portions 121.

When the lower mandrel 21 and the upper mandrel 22 are rotated by the rotating mechanism 31, the workpiece 100' rotates accordingly. As the roller 41 is pressed against the outer peripheral surface 120b' of the precursory rim 120' of the workpiece 100' in this state, the flow forming process is accomplished.

The workpiece 100' after the flow forming process are shown in FIG. 19 and FIG. 20. FIG. 19 and FIG. 20 are a left side view and a right side view, respectively, schematically showing the workpiece 100' after the flow forming process. The flow forming process has caused plastic deformation of the precursory rim 120'; more specifically, the precursory rim 120' has been stretched along the axial direction while being also thinned.

Next, a heat treatment is performed. More specifically, a solution treatment, a quenching process, and an artificial aging process are performed in this order (T6 heat treatment).

Thereafter, a cutting process is performed. Through the cutting process, the wheel-shaft insertion hole 111 and the like are formed, and also their dimensions are adjusted. At this point, the plurality of stepped portions 121 on the inner peripheral surface 120a' of the precursory rim 120' are removed. In this manner, the wheel 100 is obtained. Note that the wheel-shaft insertion hole 111 does not need to be formed via a cutting process. For example, at the step of providing the workpiece 100', a workpiece 100' that already has a wheel-shaft insertion hole 111 may be provided.

In the example described above, within the inner peripheral surface 120a' of the precursory rim 120' of the intermediate product (workpiece) 100' provided, each of the region (first region) R1 to abut with the lower mandrel (first mandrel) 21 and the region (second region) R2 to abut with the upper mandrel (second mandrel) 22 includes at least one stepped portion 121 protruding inwardly along the radial direction of the workpiece 100'. Because of such a stepped portion(s) 121 being provided on the inner peripheral surface 120a' of the precursory rim 120', the torque from the lower mandrel 21 and the upper mandrel 22 being rotated by the rotating mechanism 31 can be sufficiently transmitted to the workpiece 100'. In other words, the stepped portion(s) 121 enables clamping of the workpiece 100'. Since this makes it unnecessary to rely on the precursory hub 110' or the precursory spoke 130' for the clamping of the workpiece 100', it becomes possible to produce the wheel 100 in such a manner that clamp scars will not be left on the hub 110 and the spoke 130. For example, since the at least one stepped portion 121 including a clamping surface is removed at the step of performing a cutting process, no clamp scars will be left on the final product (i.e., the wheel 100 for straddled vehicles).

Note that the number of stepped portions 121 in each of the first region R1 and the second region R2 is not limited to what is illustrated in FIG. 13 and FIG. 14. It suffices if at least one stepped portion 121 is provided in each of the first region R1 and the second region R2.

Another exemplary configuration of the stepped portion 121 is shown in FIG. 21 and FIG. 22. In the example shown in FIG. 21 and FIG. 22, only one stepped portion 121 is provided in each of the first region R1 and the second region R2. Such a configuration also allows the wheel 100 to be produced without leaving clamp scars on the hub 110 and the spoke 130.

Still another exemplary configuration of the stepped portion 121 is shown in FIG. 23, FIG. 24, FIG. 25 and FIG. 26. In the example shown in FIG. 23 to FIG. 26, in each of the first region R1 and the second region R2, one stepped portion 121 is formed along the entire circumference along the circumferential direction of the workpiece 100'. In this case, an upper surface (i.e., a surface of the workpiece 100' facing outward along the axial direction) 121u of the stepped portion 121 has an annular shape, this upper surface 121u functioning as a clamping surface. Specifically, clamping of the workpiece 100' is achieved by utilizing a frictional force occurring between the upper surface (clamping surface) 121u of the stepped portion 121 and the abutting surface (i.e., the first abutting surface 21a of the lower mandrel 21 or the second abutting surface 22a of the upper mandrel 22) of each mandrel pressed against the upper surface 121u.

In the case where such a stepped portion 121 (a stepped portion 121 being formed along the entire circumference along the circumferential direction of the workpiece 100') are provided in each of the first region R1 and the second region R2 of the inner peripheral surface 120a' of the precursory rim 120', there is an advantage in that the workpiece 100' can be easily set to the flow forming apparatus 10.

On the other hand, as was illustrated in FIG. 13 and FIG. 14, etc., when a plurality of stepped portions 121 are formed discretely along the circumferential direction of the workpiece 100', the torque from the mandrel (the lower mandrel 21 or the upper mandrel 22) can be received on a partial side surface (a side surface oriented in the circumferential direction of the workpiece 100') of each stepped portion 121, so that not only the upper surface 121u of each stepped portion 121 but also the partial side surface functions as a clamping surface.

In the case where a plurality of stepped portions 121 are provided on the inner peripheral surface 120a' of the precursory rim 120', the workpiece 100' can be prevented from slipping against each mandrel. Moreover, a smaller amount of metal material is needed to form the workpiece 100' than in the case where one stepped portion 121 is formed continuously along the entire circumference.

Each of the first abutting surface 21a of the lower mandrel 21 and the second abutting surface 22a of the upper mandrel 22 is preferably shaped so as to correspond to at least one stepped portion 121 of the workpiece 100'. Specifically, as is illustrated, each of the first abutting surface 21a of the lower mandrel 21 and the second abutting surface 22a of the upper mandrel 22 preferably includes at least one engaging portion 23 to engage with at least one stepped portion 121.

In the step of providing the workpiece 100', the workpiece 100' can be formed from a metal material by a gravity casting technique. Employing a gravity casting technique provides an advantage of reducing the weight of relatively large wheels because it is easy to form a hollow structure by utilizing a core.

### [aluminum alloy]

Preferable compositions for the aluminum alloy to be used as the material of the wheel 100 will be described.

Preferably, the aluminum alloy contains silicon (Si) in an amount of not less than 5.0 mass% and not more than 7.5 mass%, magnesium (Mg) in an amount of not less than 0.40 mass% and not more than 0.90 mass%, and aluminum (Al) and inevitable impurities as a balance.

When the percentage content of Si is 5.0 mass% or more, castability (e.g., melt fluidity) can be adequately improved. The influence of the percentage content of Si on the melt fluidity is disclosed in Kitaoka and 2 others, "Al-Si type alloys", Light Metals, 1988, pp.426-446 (hereinafter "Non-Patent Document 1"), for example. Non-Patent Document 1 states that, for example, given a constant pour point, lowest fluidity results when the percentage content of Si is 2 to 3 mass%. On the other hand, if the percentage content of Si is too high, toughness may lower. When the percentage content of Si is 7.5 mass% or less, a decrease in toughness can be suppressed.

Moreover, since Mg yields a deposition (Mg2Si) with Si, when the percentage content of Mg is 0.40 mass% or more, tensile strength and proof stress can be improved. However, if the percentage content of Mg is too high, elongation may lower. When the percentage content of Mg is 0.90 mass% or less, a decrease in elongation due to Mg can be kept at an insignificant level.

Thus, an aluminum alloy having the aforementioned composition has good castability, as well as good tensile strength and proof stress. Good castability makes it easier to realize a complicated shape (e.g., the shape of a vehicle wheel) or a thin-walled shape, even by using a gravity casting technique. Goode tensile strength and proof stress make it possible to provide a sufficient strength even in the case of a complicated shape or a thin-walled shape.

As has already been described, as the amount of Mg added to the aluminum alloy is increased, tensile strength and proof stress may improve, but elongation (toughness) tends to lower. When a flow forming process is performed for the product (intermediate product) after casting (e.g., gravity casting), the metallographic structure changes through plastic deformation (or more specifically, the metallographic structure becomes stretched out to create a metal flow) at the site(s) which have been subjected to the flow forming process; as a result, elongation improves, thus to compensate for a decrease in elongation that is ascribable to the increased amount of Mg added. Therefore, an aluminum alloy having the aforementioned composition can be suitably used for vehicle wheels that are produced through a combination of a gravity casting technique and a flow forming process.

If the percentage content of Cu is too high, elongation may lower. Therefore, the percentage content of Cu is preferably 0.20 mass% or less.

The percentage content of Fe is preferably 0.20 mass% or less. If the percentage content of Fe is too high, toughness may lower. When the percentage content of Fe is 0.20 mass% or less, a decrease in toughness that is ascribable to Fe can be suppressed. From the standpoint of suppressing a decrease in toughness, it is more preferable that the percentage content of Fe is 0.15 mass% or less.

The percentage content of Ti is preferably 0.20 mass% or less. If the percentage content of Ti is too high, a decrease in toughness may be caused. When the percentage content of Ti is 0.20 mass% or less, a decrease in toughness that is ascribable to Ti can be suppressed.

When the aluminum alloy further contains Na in an amount of not less than 0.002 mass% and not more than 0.01 mass%, or Sr in an amount of not less than 0.005 mass% and not more than 0.03 mass%, modification (microstructuring of the eutectic Si phase) can be suitably achieved.

Now, results of studying influences of changes in the percentage content of Si, Mg, etc., in the aluminum alloy on tensile strength, proof stress, and elongation (toughness) will be described. In the following, any Example in which Si is not in the range of not less than 5.0 mass% and not more than 7.5 mass% and any Example in which Mg is not in the range of not less than 0.40 mass% and not more than 0.90 mass% is indicated as "Reference Example" for ease of understanding.

### <Si percentage content>

Table 1 shows the compositions and measurement results of tensile strength, proof stress, and elongation for aluminum alloys of Examples 1 to 3 and Reference Examples 1 to 3. As for elongation, the case where a flow forming process was not performed for the sample (indicated as "w/o FF") and the case where a flow forming process was performed for the sample (indicated as "w/ FF") are also shown. Also, for Examples 1 to 3 and Reference Example 3, their relationship between the percentage content of Si and tensile strength and proof stress is shown in FIG. 27, and their relationship between the percentage content of Si and elongation is shown in FIG. 28. In the following, a preferable tensile strength of 300 MPa or more and a preferable proof stress of 250 MPa or more are assumed, and a preferable elongation (in the case of not performing a flow forming process) of 3% or more and a preferable elongation (in the case of performing a flow forming process) of 5% or more are assumed.

**[Table 1]**

| | composition ( mass%) | | | | | | | | measurement results | | | |
|---|---|---|---|---|---|---|---|---|---|---|---|---|
| | | | | | | | | | tensile strength | proof stress | elongation (%) | |
| | Cu | Si | Mg | Fe | Ti | Na | Sr | Al | (MPa) | (MPa) | w/o FF | w/ FF |
| Reference Example 1 | 0.00 | **4.5** | 0.70 | 0.12 | 0.11 | 0.000 | 0.013 | balance | 298 | 265 | 5.8 | 8.0 |
| Reference Example 2 | 0.00 | **4.8** | 0.68 | 0.11 | 0.12 | 0.000 | 0.014 | balance | 305 | 266 | 5.5 | 7.8 |
| Example 1 | 0.00 | **5.8** | 0.71 | 0.09 | 0.12 | 0.000 | 0.009 | balance | 310 | 270 | 5.4 | 7.6 |
| Example 2 | 0.00 | **6.9** | 0.70 | 0.11 | 0.10 | 0.000 | 0.010 | balance | 319 | 275 | 5.2 | 7.3 |
| Example 3 | 0.00 | **7.3** | 0.68 | 0.12 | 0.12 | 0.000 | 0.010 | balance | 321 | 278 | 5.0 | 7.1 |
| Reference Example 3 | 0.00 | **8.0** | 0.72 | 0.12 | 0.10 | 0.000 | 0.013 | balance | 322 | 282 | 2.5 | 4.3 |

As can be seen from Table 1 and FIG. 27 and FIG. 28, in Examples 1 to 3, preferable levels are attained in all of tensile strength, proof stress, and elongation. On the other hand, in Reference Example 3, where the percentage content of Si is 8.0 mass% (i.e., above 7.5 mass%), elongation is insufficient and toughness is poor, as can be seen from Table 1 and FIG. 28.

### <Mg percentage content>

Table 2 shows the compositions and measurement results of tensile strength, proof stress, and elongation for aluminum alloys of Examples 3 to 7 and Reference Examples 4 and 5. Also, for Examples 3 to 7 and Reference Examples 4 and 5, their relationship between the percentage content of Mg and tensile strength and proof stress is shown in FIG. 29, and their relationship between the percentage content of Mg and elongation is shown in FIG. 30.

**[Table 2]**

| influences of Mg percentage content | | | | | | | | | | | | |
|---|---|---|---|---|---|---|---|---|---|---|---|---|
| | composition ( mass%) | | | | | | | | measurement results | | | |
| | | | | | | | | | tensile strength | proof stress | elongation (%) | |
| | Cu | Si | Mg | Fe | Ti | Na | Sr | Al | (MPa) | (MPa) | w/o FF | w/ FF |
| Reference Example 4 | 0.00 | 7.2 | **0.35** | 0.10 | 0.11 | 0.000 | 0.010 | balance | 278 | 230 | 9.8 | 12.0 |
| Example 4 | 0.00 | 7.2 | **0.40** | 0.09 | 0.12 | 0.000 | 0.013 | balance | 310 | 252 | 9.0 | 11.7 |
| Example 5 | 0.00 | 6.9 | **0.51** | 0.09 | 0.11 | 0.000 | 0.015 | balance | 325 | 264 | 7.5 | 10.0 |
| Example 6 | 0.00 | 7.1 | **0.62** | 0.11 | 0.11 | 0.000 | 0.013 | balance | 324 | 278 | 6.0 | 8.0 |
| Example 3 | 0.00 | 7.3 | **0.68** | 0.12 | 0.12 | 0.000 | 0.010 | balance | 321 | 278 | 5.0 | 7.1 |
| Example 7 | 0.00 | 6.9 | **0.89** | 0.12 | 0.11 | 0.000 | 0.015 | balance | 319 | 280 | 3.5 | 5.0 |
| Reference Example 5 | 0.00 | 7.0 | **0.95** | 0.11 | 0.10 | 0.000 | 0.015 | balance | 321 | 283 | 2.0 | 3.5 |

As can be seen from Table 2 and FIG. 29 and FIG. 30, in Examples 3 to 7, preferable levels are attained in all of tensile strength, proof stress, and elongation. On the other hand, in Reference Example 4, where the percentage content of Mg is 0.35 mass% (i.e., below 0.40 mass%), tensile strength and proof stress are insufficient, as can be seen from Table 2 and FIG. 29. Moreover, in Reference Example 5, where the percentage content of Mg is 0.95 mass% (i.e., above 0.90 mass%), elongation is insufficient, as can be seen from Table 2 and FIG. 30.

### <Cu percentage content>

Table 3 shows the compositions and measurement results of tensile strength, proof stress, and elongation for aluminum alloys of Examples 3, 8 and 9. Also, for Examples 3, 8 and 9, their relationship between the percentage content of Cu and tensile strength and proof stress is shown in FIG. 31, and their relationship between the percentage content of Cu and elongation is shown in FIG. 32.

**[Table 3]**

| influences of Cu percentage content | | | | | | | | | | | | |
|---|---|---|---|---|---|---|---|---|---|---|---|---|
| | composition ( mass%) | | | | | | | | measurement results | | | |
| | | | | | | | | | tensile strength | proof stress | elongation (%) | |
| | Cu | Si | Mg | Fe | Ti | Na | Sr | Al | (MPa) | (MPa) | w/o FF | w/ FF |
| Example 3 | **0.00** | 7.3 | 0.68 | 0.12 | 0.12 | 0.000 | 0.010 | balance | 321 | 278 | 5.0 | 7.1 |
| Example 8 | **0.20** | 7.0 | 0.70 | 0.11 | 0.10 | 0.000 | 0.012 | balance | 331 | 285 | 3.2 | 5.4 |
| Example 9 | **0.25** | 7.0 | 0.71 | 0.11 | 0.11 | 0.000 | 0.015 | balance | 333 | 290 | 2.5 | 3.9 |

As can be seen from Table 3 and FIG. 31 and FIG. 32, in Examples 3 and 8, preferable levels are attained in all of tensile strength, proof stress, and elongation. On the other hand, in Example 9, where the percentage content of Cu is 0.25 mass% (i.e., above 0.20 mass%), elongation is smaller than in Examples 3 and 8, as can be seen from Table 3 and FIG. 32.

### <Fe percentage content>

Table 4 shows the compositions and measurement results of tensile strength, proof stress, and elongation for aluminum alloys of Examples 3, 10 and 11. Also, for Examples 3, 10 and 11, their relationship between the percentage content of Fe and tensile strength and proof stress is shown in FIG. 33, and their relationship between the percentage content of Fe and elongation is shown in FIG. 34.

**[Table 4]**

| influences of Fe percentage content | | | | | | | | | | | | |
|---|---|---|---|---|---|---|---|---|---|---|---|---|
| | composition ( mass%) | | | | | | | | measurement results | | | |
| | | | | | | | | | tensile strength | proof stress | elongation (%) | |
| | Cu | Si | Mg | Fe | Ti | Na | Sr | Al | (MPa) | (MPa) | w/o FF | w/ FF |
| Example 3 | 0.00 | 7.3 | 0.68 | **0.12** | 0.12 | 0.000 | 0.010 | balance | 321 | 278 | 5.0 | 7.1 |
| Example 10 | 0.00 | 7.3 | 0.70 | **0.20** | 0.11 | 0.000 | 0.014 | balance | 325 | 285 | 3.1 | 5.0 |
| Example 11 | 0.00 | 7.2 | 0.70 | **0.24** | 0.11 | 0.000 | 0.012 | balance | 328 | 286 | 1.5 | 3.0 |

As can be seen from Table 4 and FIG. 33 and FIG. 34, in Examples 3 and 10, preferable levels are attained in all of tensile strength, proof stress, and elongation. On the other hand, in Example 11, where the percentage content of Fe is 0.24 mass% (i.e., above 0.20 mass%), elongation is smaller (i.e., toughness is lower) than in Examples 3 and 10, as can be seen from Table 4 and FIG. 34.

### <Ti percentage content>

Table 5 shows the compositions and measurement results of tensile strength, proof stress, and elongation for aluminum alloys of Examples 3, 12 and 13. Also, for Examples 3, 12 and 13, their relationship between the percentage content of Ti and tensile strength and proof stress is shown in FIG. 35, and their relationship between the percentage content of Ti and elongation is shown in FIG. 36.

**[Table 5]**

| influences of Ti percentage content | | | | | | | | | | | | |
|---|---|---|---|---|---|---|---|---|---|---|---|---|
| | composition ( mass%) | | | | | | | | measurement results | | | |
| | | | | | | | | | tensile strength | proof stress | elongation (%) | |
| | Cu | Si | Mg | Fe | Ti | Na | Sr | Al | (MPa) | (MPa) | w/o FF | w/ FF |
| Example 3 | 0.00 | 7.3 | 0.68 | 0.12 | **0.12** | 0.000 | 0.010 | balance | 321 | 278 | 5.0 | 7.1 |
| Example 12 | 0.00 | 7.4 | 0.72 | 0.11 | **0.19** | 0.000 | 0.009 | balance | 324 | 286 | 4.0 | 5.3 |
| Example 13 | 0.00 | 7.5 | 0.71 | 0.12 | **0.24** | 0.000 | 0.011 | balance | 330 | 290 | 2.8 | 4.0 |

As can be seen from Table 5 and FIG. 35 and FIG. 36, in Examples 3 and 12, preferable levels are attained in all of tensile strength, proof stress, and elongation. On the other hand, in Example 13, where the percentage content of Ti is 0.24 mass% (i.e., above 0.20 mass%), elongation is smaller (i.e., toughness is lower) than in Examples 3 and 10, as can be seen from Table 5 and FIG. 36.

### <Na and Sr percentage contents>

Table 6 shows the compositions and measurement results of tensile strength, proof stress, and elongation for aluminum alloys of Examples 3, and 14 to 20. Also, for Examples 14 to 17, their relationship between the percentage content of Na and tensile strength and proof stress is shown in FIG. 37, and their relationship between the percentage content of Na and elongation is shown in FIG. 38. Also, for Examples 3, 14, and 18 to 20, their relationship between the percentage content of Sr and tensile strength and proof stress is shown in FIG. 39, and their relationship between the percentage content of Sr and elongation is shown in FIG. 40.

**[Table 6]**

| influences of Na and Sr percentage contents | | | | | | | | | | | | |
|---|---|---|---|---|---|---|---|---|---|---|---|---|
| | composition ( mass%) | | | | | | | | measurement results | | | |
| | | | | | | | | | tensile strength | proof stress | elongation (%) | |
| | Cu | Si | Mg | Fe | Ti | Na | Sr | Al | (MPa) | (MPa) | w/o FF | w/ FF |
| Example 14 | 0.00 | 7.2 | 0.73 | 0.10 | 0.11 | **0.000** | **0.000** | balance | 322 | 280 | 2.5 | 3.7 |
| Example 15 | 0.00 | 7.0 | 0.70 | 0.10 | 0.12 | **0.002** | **0.000** | balance | 320 | 280 | 3.0 | 5.2 |
| Example 16 | 0.00 | 7.3 | 0.69 | 0.12 | 0.12 | **0.012** | **0.000** | balance | 319 | 275 | 5.5 | 8.0 |
| Example 17 | 0.00 | 7.1 | 0.71 | 0.11 | 0.11 | **0.019** | **0.000** | balance | 325 | 277 | 5.7 | 7.9 |
| Example 18 | 0.00 | 7.1 | 0.70 | 0.09 | 0.12 | **0.000** | **0.005** | balance | 318 | 275 | 4.1 | 6.2 |
| Example 3 | 0.00 | 7.3 | 0.68 | 0.12 | 0.12 | **0.000** | **0.010** | balance | 321 | 278 | 5.0 | 7.1 |
| Example 19 | 0.00 | 7.2 | 0.70 | 0.12 | 0.10 | **0.000** | **0.028** | balance | 326 | 280 | 6.9 | 9.3 |
| Example 20 | 0.00 | 6.9 | 0.72 | 0.10 | 0.11 | **0.000** | **0.040** | balance | 325 | 282 | 7.0 | 9.5 |

As can be seen from Table 6 and FIG. 37 to FIG. 40, in Examples 3, and 15 to 20, preferable levels are attained in all of tensile strength, proof stress, and elongation. On the other hand, in Example 14, where neither Na nor Sr is substantially contained, elongation is smaller than in Examples 3, and 15 to 20, as can be seen from Table 6 and FIG. 38 and FIG. 40. This is presumably because modification (microstructuring of the eutectic Si phase) is not suitably achieved.

According to an embodiment of the present teaching, there is provided a method of producing a wheel for straddled vehicles that is able to adequately improve the mechanical properties of a rim. A production method according to an embodiment of the present teaching can be suitably used for the production of a wheel for various straddled vehicles, such as motorcycles.

## Claims

1. A method of producing a wheel (100) for straddled vehicles, the wheel (100) including: a hub (110) having an aperture (111) into which a wheel shaft is to be inserted; an annular rim (120); and a plurality of spokes (130) connecting the hub (110) and the rim (120), the method comprising:
step A (s1) of forming an intermediate product (100') from an aluminum alloy by using a gravity casting technique, the intermediate product (100') including a precursory hub (110'), an annular precursory rim (120'), and a plurality of precursory spokes (130') connecting the precursory hub (110') and the precursory rim (120');
step B (s2) of performing a flow forming process for the precursory rim (120') of the intermediate product (100') by using a flow forming apparatus (10), wherein, while the intermediate product (100') is rotated, at least a portion of the precursory rim (120') is drawn in a first direction (D1) and a second direction (D2), the first direction (D1) being one direction that extends from a center of the intermediate product (100') on an axial direction of the intermediate product (100'), and the second direction (D2) being an opposite direction that extends from the center of the intermediate product (100') on the axial direction of the intermediate product (100'); and
step C (s6) of, after step B (s2), performing a cutting process for the intermediate product (100') to at least complete the rim (120), wherein,
a ratio of a wall thickness (t1) of the precursory rim (120') after step B (s2) and before step C (s6) to a wall thickness (t2) of the rim (120) after step C (s6) is not less than 132% and not more than 433%.

2. The method of producing of claim 1, wherein step B (s2) is performed in such a manner that, in at least a portion of the precursory rim (120'), a ratio of the wall thickness (t1) of the precursory rim (120') after step B (s2) and before step C (s6) to a wall thickness (t2) of the precursory rim (120') before step B (s2) is 50% or less.

3. The method of producing of claim 1 or 2, wherein the flow forming apparatus (10) includes:
a first mandrel (21) having a first abutting surface (21a) that abuts with an inner peripheral surface (120a') of the precursory rim (120') of the intermediate product (100') from one direction along the axial direction of the intermediate product (100');
a second mandrel (22) having a second abutting surface (22a) that abuts with the inner peripheral surface (120a') of the precursory rim (120') of the intermediate product (100') from an opposite direction along the axial direction of the intermediate product (100');
a rotating mechanism (31) to rotate the first mandrel (21) and the second mandrel (22); and
a roller (41) to be pressed against an outer peripheral surface (120b') of the precursory rim (120') of the intermediate product (100').

4. The method of producing of claim 3, wherein, the flow forming apparatus (10) further includes a knockout ring (24) located near an outer periphery of the first mandrel (21) so as to be able to move up and down;
an upper surface of the knockout ring (24) is offset from a reference plane (p) along the first direction (D1); and
an amount of offset of an upper surface of the knockout ring (24) from the reference plane (p) is set so that the amount increases as a ratio L1/L2 increases, wherein the ratio L1/L2 is a ratio of a length L1 of the precursory rim (120') after step B (s2) and before step C (s6) as taken along the axial direction of the intermediate product (100') to a length L2 of the rim (120) after step C (s6) as taken along the axial direction of the intermediate product (100').

5. The method of producing of claim 4, wherein the ratio L1/L2 is not less than 101% and not more than 113%.

6. The method of producing of any of claims 3 to 5, wherein, the inner peripheral surface (120a') of the precursory rim (120') of the intermediate product (100') formed at step A (s1) includes a first region R1 to abut with the first abutting surface (21a) of the first mandrel (21) and a second region (R2) to abut with the second abutting surface (22a) of the second mandrel (22); and
each of the first region (R1) and the second region (R2) of the inner peripheral surface (120a') of the precursory rim (120') includes at least one stepped portion (121) protruding inwardly along a radial direction of the intermediate product (100').

7. The method of producing of claim 6, wherein the at least one stepped portion (121) is one stepped portion (121) formed along an entire circumference along a circumferential direction of the intermediate product (100').

8. The method of producing of claim 6, wherein the at least one stepped portion (121) comprises a plurality of stepped portions that are formed discretely along a circumferential direction of the intermediate product (100').

9. The method of producing of any of claims 6 to 8, wherein each of the first abutting surface (21a) of the first mandrel (21) and the second abutting surface (22a) of the second mandrel (22) includes at least one engaging portion (23) to engage with the at least one stepped portion (121).

10. The method of producing of any of claims 6 to 9, wherein the at least one stepped portion (121) is removed in step C (s6).

## Patentansprüche

1. Ein Verfahren zur Herstellung eines Rades (100) für Spreiz-Sitz-Fahrzeuge, das Rad (100) enthält: eine Nabe (110), die eine Öffnung (111) hat, in die eine Radwelle einzusetzen ist; einen ringförmigen Kranz (120); und eine Mehrzahl von Speichen (130), welche die Nabe (110) und den Kranz (120) verbinden, das Verfahren umfasst:
Schritt A (s1) des Formens eines Zwischenprodukts (100') aus einer Aluminiumlegierung unter Verwendung einer Schwerkraftgusstechnik, das Zwischenprodukt (100') enthält eine Vorläufernabe (110'), einen ringförmigen Vorläuferkranz (120') und eine Mehrzahl von Vorläuferspeichen (130'), welche die Vorläufemabe (110') und den Vorläuferkranz (120') verbinden;
Schritt B (s2) des Durchführens eines Fließformungsprozesses für den Vorläuferkranz (120') des Zwischenprodukts (100') unter Verwendung einer Fließformungsvorrichtung (10), wobei, während das Zwischenprodukt (100') gedreht wird, zumindest ein Abschnitt des Vorläuferkranzes (120') in eine erste Richtung (D1) und eine zweite Richtung (D2) gezogen wird, die erste Richtung (D1) ist eine Richtung, die sich von einer Mitte des Zwischenprodukts (100') in einer axialen Richtung des Zwischenprodukts (100') erstreckt, und die zweite Richtung (D2) ist eine entgegengesetzte Richtung, die sich von der Mitte des Zwischenprodukts (100') in der axialen Richtung des Zwischenprodukts (100') erstreckt; und
Schritt C (s6) von, nach Schritt B (s2), des Durchführens eines Schneidprozess für das Zwischenprodukt (100'), um zumindest den Kranz (120) zu vervollständigen, wobei,
ein Verhältnis der Wanddicke (t1) des Vorläuferkranzes (120') nach Schritt B (s2) und vor Schritt C (s6) zu einer Wanddicke (t2) des Kranzes (120) nach Schritt C (s6) nicht weniger als 132 % und nicht mehr als 433 % ist.

2. Das Verfahren zur Herstellung von Anspruch 1, wobei Schritt B (s2) so durchgeführt wird, dass in zumindest einem Abschnitt des Vorläuferkranzes (120') das Verhältnis der Wanddicke (t1) des Vorläuferkranzes (120') nach Schritt B (s2) und vor Schritt C (s6) zu einer Wanddicke (t2) des Vorläuferkranzes (120') vor Schritt B (s2) 50 % oder weniger beträgt.

3. Das Verfahren zur Herstellung von Anspruch 1 oder 2, wobei die Fließformungsvorrichtung (10) enthält:
einen ersten Dorn (21) mit einer ersten Anlagefläche (21a), die an einer inneren Umfangsfläche (120a') des Vorläuferkranzes (120') des Zwischenprodukts (100') aus einer Richtung entlang der axialen Richtung des Zwischenprodukts (100') anliegt;
einen zweiten Dorn (22) mit einer zweiten Anlagefläche (22a), die an der inneren Umfangsfläche (120a') des Vorläuferkranzes (120') des Zwischenprodukts (100') aus einer entgegengesetzten Richtung entlang der axialen Richtung des Zwischenprodukts (100') anliegt;
einen Drehmechanismus (31), um den ersten Dorn (21) und den zweiten Dorn (22) zu drehen; und
eine Rolle (41), die gegen eine äußere Umfangsfläche (120b') des Vorläuferkranzes (120') des Zwischenprodukts (100') gedrückt wird.

4. Das Verfahren zur Herstellung von Anspruch 3, wobei die Fließformungsvorrichtung (10) weiterhin einen Auswurfring (24) enthält, der in der Nähe eines Außenumfangs des ersten Dorns (21) angeordnet ist, so dass er in der Lage ist, sich auf und ab zu bewegen;
eine obere Fläche des Auswurfrings (24) von einer Bezugsebene (p) entlang der ersten Richtung (D1) versetzt ist; und
ein Betrag des Versatzes einer oberen Fläche des Auswurfrings (24) von der Bezugsebene (p) so eingestellt ist, dass der Betrag mit zunehmendem Verhältnis L1/L2 zunimmt, wobei das Verhältnis L1/L2 ein Verhältnis einer Länge L1 des Vorläuferkranzes (120') nach Schritt B (s2) und vor Schritt C (s6), gemessen entlang der axialen Richtung des Zwischenprodukts (100'), zu einer Länge L2 des Kranzes (120) nach Schritt C (s6), gemessen entlang der axialen Richtung des Zwischenprodukts (100'), ist.

5. Das Verfahren zur Herstellung von Anspruch 4, wobei das Verhältnis L1/L2 nicht weniger als 101 % und nicht mehr als 113 % beträgt.

6. Das Verfahren zur Herstellung von irgendeinem der Ansprüche 3 bis 5, wobei die innere Umfangsfläche (120a') des Vorläuferkranzes (120') des Zwischenprodukts (100'), das in Schritt A (s1) gebildet ist, einen ersten Bereich R1 zur Anlage an der ersten Anlagefläche (21a) des ersten Dorns (21) und einen zweiten Bereich (R2) zur Anlage an der zweiten Anlagefläche (22a) des zweiten Dorns (22) enthält; und
jeder von dem ersten Bereich (R1) und dem zweiten Bereich (R2) der inneren Umfangsfläche (120a') des Vorläuferkranzes (120') zumindest einen abgestuften Abschnitt (121) enthält, der entlang einer radialen Richtung des Zwischenprodukts (100') nach innen vorsteht.

7. Das Verfahren zur Herstellung von Anspruch 6, wobei der zumindest eine gestufte Abschnitt (121) ein gestufter Abschnitt (121) ist, der entlang eines gesamten Umfangs entlang einer Umfangsrichtung des Zwischenprodukts (100') ausgebildet ist.

8. Das Verfahren zur Herstellung von Anspruch 6, wobei der zumindest eine gestufte Abschnitt (121) eine Mehrzahl von gestuften Abschnitten umfasst, die diskret entlang einer Umfangsrichtung des Zwischenprodukts (100') ausgebildet sind.

9. Das Verfahren zur Herstellung von irgendeinem der Ansprüche 6 bis 8, wobei jede von der ersten Anlagefläche (21a) des ersten Dorns (21) und der zweiten Anlagefläche (22a) des zweiten Dorns (22) zumindest einen Eingriffsabschnitt (23) enthält, der mit dem zumindest einen abgestuften Abschnitt (121) in Eingriff ist.

10. Das Verfahren zur Herstellung von irgendeinem der Ansprüche 6 bis 9, wobei der zumindest eine gestufte Abschnitt (121) in Schritt C (s6) entfernt wird.

## Revendications

1. Procédé de fabrication d'une roue (100) pour des véhicules à selle, la roue (100) incluant un moyeu (110) comportant une ouverture (111) dans laquelle doit être inséré un arbre de roue, une jante annulaire (120) et une pluralité de rayons (130) reliant le moyeu (110) et la jante (120), le procédé comprenant :
l'étape A (s1) consistant à façonner un produit intermédiaire (100') à partir d'un alliage d'aluminium en utilisant une technique de moulage par gravité, le produit intermédiaire (100') incluant un moyeu préliminaire (110') une jante annulaire préliminaire (120') et une pluralité de rayons préliminaires (130') reliant le moyeu préliminaire (110') et la jante préliminaire (120'),
l'étape B (s2) consistant à effectuer un processus de fluotournage concernant la jante préliminaire (120') du produit intermédiaire (100') en utilisant un appareil de fluotournage (10), où, alors que le produit intermédiaire (100') est mis en rotation, au moins une partie de la jante mère (120') est étirée dans une première direction (D1) et dans une seconde direction (D2), la première direction (D1) étant une direction qui s'étend depuis le centre du produit intermédiaire (100') sur la direction axiale du produit intermédiaire (100') et la seconde direction (D2) étant la direction opposée qui s'étend depuis le centre du produit intermédiaire (100') sur la direction axiale du produit intermédiaire (100'), et
l'étape C (s6) consistant, après l'étape B (s2), à effectuer un procédé de découpe concernant le produit intermédiaire (100') pour au moins achever la jante (120), où
le rapport de l'épaisseur de paroi (t1) de la jante préliminaire (120') après l'étape B (s2) et avant l'étape C (s6) sur l'épaisseur de paroi (t2) de la jante (120) après l'étape C (s6) n'est pas inférieure à 132 % et pas supérieure à 433 %.

2. Procédé de fabrication selon la revendication 1, dans lequel l'étape B (s2) est effectuée de manière à ce que, dans au moins une partie de la jante préliminaire (120'), le rapport de l'épaisseur de paroi (t1) de la jante préliminaire (120') après l'étape B (s2) et avant l'étape C (s6) sur l'épaisseur de paroi (t2) de la jante préliminaire (120') avant l'étape B (s2) vaut 50 % ou moins.

3. Procédé de fabrication selon la revendication 1 ou la revendication 2, dans lequel l'appareil de fluotournage (10) inclut :
un premier mandrin (21) présentant une première surface de butée (21a) qui vient en butée avec la surface périphérique interne (120a') de la jante préliminaire (120') du produit intermédiaire (100') depuis une première direction le long de la direction axiale du produit intermédiaire (100'),
un second mandrin (22) présentant une seconde surface de butée ouverte 22a) qui vient en butée avec la surface périphérique interne (120a') de la jante préliminaire (120') du produit intermédiaire (100') depuis la direction opposée le long de la direction axiale du produit intermédiaire (100'),
un mécanisme de mise en rotation (31) destiné à faire tourner le premier mandrin (21) et le second mandrin (22), et
un galet (41) a pressé contre la surface périphérique interne (120b') de la jante préliminaire (120') du produit intermédiaire (100').

4. Procédé de fabrication selon la revendication 3, dans lequel l'appareil de fluotournage (10) inclut en outre une bague d'éjection (24) située à proximité de la périphérie externe du premier mandrin (21) de sorte à pouvoir effectuer un mouvement vers le haut et le bas,
la surface supérieure de la bague d'éjection (24) est décalée d'un plan de référence (p) le long de la première direction (D1), et
la valeur de décalage de la surface supérieure de la bague d'éjection (24) par rapport au plan de référence (p) est établie de sorte à ce que la valeur augmente à mesure que le rapport L1/L2 augmente, le rapport L1/L2 étant le rapport de la longueur L1 de la jante préliminaire (120') après l'étape B (s2) et avant l'étape C (s6) telle qu'elle est prise le long de la direction axiale du produit intermédiaire (100') sur la longueur L2 de la jante (120) après l'étape C (s6) telle qu'elle est prise le long de la direction axiale du produit intermédiaire (100').

5. Procédé de fabrication selon la revendication 4, dans lequel le rapport L1/L2 n'est pas inférieur à 101 % et pas supérieur à 113 %.

6. Procédé de fabrication selon l'une quelconque des revendications 3 à 5, dans lequel la surface périphérique interne (120a') de la jante préliminaire (120') du produit intermédiaire (100') formé à l'étape A (s1) inclut une première zone R1 destinée à venir en butée avec la première surface de butée (21a) du premier mandrin (21) et une seconde zone (R2) destinée à venir en butée avec la seconde surface de butée (22a) du second mandrin (22), et
chacune de la première zone (R1) et de la seconde zone (R2) de la surface périphérique interne (120a') de la jante préliminaire (120') inclut au moins un échelon (121) dépassant vers l'intérieur le long d'une direction radiale du produit intermédiaire (100').

7. Procédé de fabrication selon la revendication 6, dans lequel le ou les selon (121) sont un échelon (121) formée sur toute la circonférence le long de la direction circonférentielle du produit intermédiaire (100').

8. Procédé de fabrication selon la revendication 6, dans lequel le ou les échelons (121) comprennent une pluralité de parties en échelon qui sont formées de façon discrète le long de la direction circonférentielle du produit intermédiaire (100').

9. Procédé de fabrication selon l'une quelconque des revendications 6 à 8, dans lequel chacune de la première surface de butée (21a) du premier mandrin (21) et de la seconde surface de butée (22a) du second mandrin (22) inclut au moins un organe d'engrènement (23) destiné à se mettre en prise avec le ou les échelons (121)

10. Procédé de fabrication selon l'une quelconque des revendications 6 à 9, dans lequel le ou les échelons (121) sont éliminés à l'étape C (s6).
